

# UNITED STATES PATENT OFFICE.

LOUIS E. LEVI, OF MILWAUKEE, WISCONSIN, ASSIGNOR TO PFISTER & VOGEL LEATHER COMPANY, OF MILWAUKEE, WISCONSIN, A CORPORATION OF WISCONSIN.

## PROCESS OF TAWING AND TANNING.

1,135,977.

Specification of Letters Patent. Patented Apr. 13, 1915.

No Drawing.

Application filed December 29, 1913. Serial No. 809,221.

To all whom it may concern:

Be it known that I, LOUIS E. LEVI, a citizen of the United States, and resident of Milwaukee, in the county of Milwaukee and 5 State of Wisconsin, have invented new and useful Improvements in Processes of Tawing and Tanning, of which the following is a description.

It is a well known fact that compounds of 10 chromium or other mineral salts have been used for the purpose of tawing or tanning hides and skins in order to convert the animal fiber into leather but the employment of such substances has been accompanied by 15 certain disadvantages, namely:—First, the leather is always soft; second, the process of tawing or tanning consumes too much time; third, the wearing quality of the leather is poor so that the life thereof is short; fourth, 20 the cost of manufacture is too high.

The process hereinafter described has for its object to obviate the above mentioned disadvantages.

The hides and skins are prepared in the 25 usual well known manner, that is, soaking, dehairing, washing, deliming, washing, pressing and pickling. The hides and skins are taken from the salt and sulfuric acid pickle or from the formaldehyde pickle, and 30 pressed and placed in the drum or vat with or without the addition of salt (NaCl) or glauber salt (Na<sub>2</sub>SO<sub>4</sub>) with sufficient water to float the stock, in case drum tannage is used, or sufficient water to cover the stock 35 in case vat tannage is used. Then, any of the following compounds are gradually added, or any combination of them, and the amount added in usual cases is from three to four per cent. of the pressed pickled 40 weight of the stock. When the stock is struck through it is placed in a vat or drum with a solution of one of the following substances:—Thiosulfate of soda, bisulfite of soda, bicarbonate of soda or carbonate of soda. Then it is washed, drained and finished in the usual manner. If the stock is intended for sole leather, to be hard and firm, it is simply oiled off on the grain and flesh. For softer upper leather the stock is 45 impregnated with greases or fat liquors as this term is generally understood among tanners and curriers. The following are the compounds used by me in tawing or tanning hides or skins, either alone or in combina-

tion, in the presence or absence of an acid. 55 In the manufacture of the compounds sodium or potassium salts are used:

Ferric chromate such as:—



Basic ferric chromate such as:—



Ferric sulfo chromates such as:—



and the like.

Basic ferric sulfo chromates such as:—



and the like. 90

Ferric chloro chromates

Basic ferric chloro chromates

Ferric chloro sulfo chromates

Basic ferric chloro sulfo chromates

All are made like the above sulfo salts by 95 using the chlorids and a combination of the chlorids and sulfates of the different metals.

I have also discovered that compounds can also be made by the action of chromic acid (CrO<sub>3</sub>) upon the basic ferric compounds 100 such as the following:



and the like which are excellent tanning or tawing compounds.

What I claim as new and desire to secure by Letters Patent is:

1. The process of tanning consisting of immersing hides in a solution of a non-acid ferric chromate.

2. The process of tanning consisting of immersing hides in a solution of a non-acid substituted ferric chromate.

In testimony whereof, I affix my signature, in presence of two witnesses.

LOUIS E. LEVI.

Witnesses:

R. S. C. CALDWELL,  
KATHERINE HOLT.

Copies of this patent may be obtained for five cents each, by addressing the "Commissioner of Patents, Washington, D. C."